

Oct. 8, 1968

W. A. TOMPKINS

3,404,525

LOW-TORQUE MULTIFILAMENT COMPACT YARN

Filed Sept. 1, 1966

2 Sheets-Sheet 1



Inventor  
WILLIAM ARTHUR TOMPKINS

By  
Cushman, Leiby & Cushman  
Attorneys

Oct. 8, 1968

W. A. TOMPKINS

3,404,525

LOW-TORQUE MULTIFILAMENT COMPACT YARN

Filed Sept. 1, 1966

2 Sheets-Sheet 2

Fig. 4.



Fig. 5.



WILLIAM ARTHUR <sup>Inventor</sup> TOMPKINS

Cushman, Darby & Cushman  
By  
Attorneys

**1**

3,404,525

**LOW-TORQUE MULTIFILAMENT COMPACT  
YARN**William Arthur Tompkins, Usk, England, assignor to  
Imperial Chemical Industries Limited, London, Eng-  
land

Filed Sept. 1, 1966, Ser. No. 576,766

Claims priority, application Great Britain, Sept. 10, 1965,  
38,689/65

4 Claims. (Cl. 57—149)

**ABSTRACT OF THE DISCLOSURE**

A compact multifilament yarn wherein the filaments are parallel and which exhibits a low torque of between .25 and 2.5 turns per inch and has no twist and no crimp. Also, a yarn having the above specified torque and also a twist of .25 turn per inch in the same direction as the torque.

The invention concerns low-torque multifilament compact yarn.

Torque in a yarn results from torsional stress induced by twisting; and it is conveniently expressed as the turns per inch of twist-liveliness measured in the yarn. Owing to the fact that torque decays at a rate dependent on, inter alia, the value of the initial torque and the conditions of yarn storage, the values of torque referred to herein are those present in the yarn when the measurements were made approximately 4 hours after production of the yarn. The values would be significantly different if the measurements were taken after the yarn had been stored for, say, 30 days; for instance a torque of 2.5 turns per inch in 45 denier/15 filament nylon 66 yarn can decay to one of 2.0 turns per inch over that period.

A "compact" yarn is one which by virtue of interfilamentary cohesion is manipulable as an entity without defects arising from handling, running, etc.

The traditional manner of compacting a multifilament yarn has been by twisting i.e. by the insertion of unidirectional twist. Twisting, however, imposes limitations on the productivity of yarn production processes, and is not comparable in this respect with pure winding.

Hence, attention has recently been paid to other means of compacting, as for instance alternating twist, filament interlacing and filament adhesion.

The invention concerns a novel multifilament compact yarn, and the method of producing it.

According to the invention, a multifilament compact yarn is characterised by the absence of any substantial unidirectional twist and the presence of from 0.25 to 2.5 turns per inch unidirectional torque. The narrow range of torque is called for by the need to have sufficient torque to cause the filaments to bind together but not so much as to lead to handling defects, such as looping or snarling during subsequent pining, or to fabric defects, such as spiralling of knitted fabric panels for stockings, due to excessive twist-liveliness.

By the "absence of any substantial unidirectional twist," we mean that there shall be twist of, or less than, the minimum value of "producer twist" for the yarn in question, generally 0.25 turn per inch or less.

Experiments have shown that with 60 denier/20 filament and 70 denier/34 filament yarn of polyhexamethylene adipamide a truly compact yarn is obtained, which will not give rise to a tendency to looping in the most significant after-treatment of pining, without twist and at a torque of 1.5 turns per inch. Such yarns have been used as weft in the manufacture of woven fabrics having no faults attributable to the handling properties of the yarn. With these particular yarns any increase much

**2**

beyond about 2.0 turns per inch led to an incidence of looping or snarling defects at pining (say, in 1 out of every 10 pines); and a decrease below about 0.5 led to handling difficulties due to filament separation, especially at low speeds (e.g. up to 200 feet/minute). Transfer of the yarns from one package to another at speeds up to 2,400 feet/minute has been achieved satisfactorily at normal yarn transfer tensions when the torque is between 0.5 turn per inch and 2.5 turns per inch.

Torque of the low degree in question may be introduced in a number of ways, but the most convenient, from the point of view of productivity, involves the imparting of false twist to the running yarn while it is hot.

Conveniently, such low-torque false twist can be imparted during the drawing process carried out on multifilament yarns of synthetic polymeric material, as for instance polyamide, polyester and polypropylene material. For instance, the false twist can be imparted actually while the yarn is being drawn; or it can be imparted subsequently to the drawing having been effected but prior to wind-up thereafter.

In such drawing process, undrawn yarn is fed into a drawing zone at a predetermined rate, the point of draw normally being localized on a snubbing-pin which is preferably heated, and the yarn is drawn by the action of draw rolls operating at a multiple of the predetermined rate. The yarn is then wound up, either with or without the imparting of a low degree of twist.

The appropriate low degree of torque can be obtained from a range of combinations of twist insertion and setting, i.e. from low twist with a high degree of set (e.g. using a heated metal snubbing-pin) to high twist with a low degree of set (e.g. with a cold metal or ceramic snubbing-pin, or no pin at all and a feed roll).

According to British Patent No. 890,053, false twist may be imparted during the drawing process, by passing the yarn, en route from the snubbing-pin to the draw roll, partially around and in frictional contact with a convex-surfaced flange fitted to one end of the draw roll, whereby the yarn is caused to roll about its axis. The flange may be made, for instance, of neoprene of 78° shore hardness; but observing that only a low degree of false twist is needed to be imparted, as opposed to the degree required for crimping as disclosed in the aforesaid specification, other more durable materials such as chromed steel may be used, with a larger angle of wrap of the yarn in contact with the flange than would be required with materials of a higher coefficient of friction.

It is also possible to impart false twist by means of a twist-tube false twister, either of the sort which acts directly on the yarn by friction or of the sort which causes rotation of the yarn by wrapping it around a pin or roller.

The yarn according to the invention is compact but with only a negligible amount of filament interlacing, and with sensibly zero unidirectional twist. The filaments are effectively parallel to one another and to the length direction of the yarn.

If desired, in order to reduce the residual shrinkage in the yarn, normally to at least half its normal value, a heat-relaxing treatment may be carried out on the yarn, concomitantly with false twisting, by passing the yarn over or through a heating device. Such device may, if desired, comprise a jet supplied with heated gas, such as hot air or steam, under pressure, so long as sensibly no filament interlacing or twisting is involved in its use.

Alternatively, the heating device may comprise a cylindrical convection heater supplied with e.g. hot air or steam; or it may comprise a contact heater, preferably a curved plate or plates heated electrically to the desired temperature. It is preferred to utilize the heat imparted for this heat-relaxation treatment for the pre-false-twist-

ing heating also; but if such heat-relaxing is carried-out subsequently to de-twisting, it will be necessary to impart a higher degree of false twist than normal, as the relaxation treatment tends to accelerate the torque decay.

A normal amount of twist is about double that of the torque desired, assuming thorough setting of the twist.

The yarn prior to false twisting is in its normal condition, i.e. it will have the normal amount of spinning finish thereon. It is unnecessary and undesirable to have any solvent applied to the yarn before false-twisting, unless the yarn material is of a kind which will not allow of the setting of twist with heat alone or with heat combined with the action of drawing.

The invention is applicable to all multifilament yarns of any material capable of being set, notably the synthetic yarn materials. Thus, although 60/20 and 70/34 yarns have been specifically referred to above, the yarns may be sheerer, as for instance 15/3 or 20/7, or they may be heavier, as for instance 205/34. The polyamides, polyesters and polypropylenes represent the presently most useful yarn materials.

In view of the low torque present in the yarn, it is necessary to withdraw the yarn from its package at a sufficient tension to prevent snarling; but this does not present any difficulty, as the tension will never be likely to be higher than that normally required in any textile process utilizing the yarn as a supply. A low torque may be used to supplement a low twist, so that the combined compacting effect of torque and twist is adequate for the purpose in hand, the values of both being lower than those required when either torque or twist alone is used for compacting of the yarn in question.

The invention will now be described by reference to the accompanying drawings, in which—

FIGURE 1 is a diagram of drawing apparatus incorporating a rubber flange on one end of the draw roll;

FIGURE 1a is a side elevational view of the draw roll of FIGURE 1;

FIGURE 2 is a diagram of drawing apparatus with provision for the false-twisting of the drawn yarn and its relaxation in a cylindrical heater;

FIGURE 3 is a diagram of drawing apparatus with provision for the false-twisting of the drawn yarn and its relaxation by contact with a contact heater;

FIGURE 4 is a diagram of drawing apparatus with provision for heating and false-twisting the yarn whilst it is being drawn; and

FIGURE 5 is a diagram of a modified form of the apparatus of FIGURE 1.

In the drawings, the same reference numerals have been

tween which sets of rolls the yarn, Y, is drawn, the point of draw being localized by the snubbing-pin 11, which can be either ceramic or metal and around which the yarn is wrapped with two turns. At one end of draw roll 5 is attached curved flange 9, which may be of rubber or of metal; and the yarn path between snubbing-pin 11 and draw roll 5 makes an angle  $\theta$  with the perpendicular to the axis of the draw roll, the value of  $\theta$  affecting the amount of torque to be induced by the false twisting action of the flange on the yarn.

In FIGURE 2, a hot air heater 13 with a false twister 19 is positioned downstream of draw roll 5; and the drawn yarn is both heat-relaxed and false twisted before being passed via guide 19 to a winding mechanism (not shown).

The arrangement of FIGURE 3 is similar to that of FIGURE 2 save that the yarn is relaxed by an amount controlled by the degree of step-down of a stepped draw roll 5, 5a combined with its stepped separator roll 7, 7a. The yarn is fed into the drawing zone by feed roll 1 and 20 nip roll 1a. The heat-relaxing heater in this case is a contact heater 21 of the two-sided (or "pyramid") type, the yarn passing in contact with a heated surface of the heater up one side, around pulley wheel 23 and then down the other side of the heater in contact with a heated surface 25 thereof.

In FIGURE 4, the torque is induced by means of a false twister 17 within the drawing span, the heater (to heat the yarn upstream of the false twister) in this case being a single-sided contact heater 27. The yarn is fed into the 30 drawing zone by feed roll 1 with nip roll 1a, the yarn first being taken on a partial wrap around feed roll 1, thence around grooved ceramic pin 25 and finally between the nip of rolls 1 and 1a.

The arrangement of apparatus shown in FIGURE 5, 35 which is especially for use with heavier denier yarn of "Terylene" (registered trademark) polyester fibre, is essentially similar to that of FIGURES 1 and 1a, but with the addition of adjustable ceramic pin 29 between an electrically-heated metal snubbing-pin 11, having electric leads 31, and the draw roll 5.

The following examples illustrate but do not limit the invention.

#### Example I

Multifilament yarns of polyhexamethylene adipamide, of the deniers and filament numbers indicated, were drawn, and torque was induced in them, by the apparatus of FIGURES 1 and 1a, the draw roll being provided with a rubber flange of 20 cms. diameter and 5 cms. cross-sectional radius of curvature (see FIGURE 1a) and shore hardness 87-90 fitted on a draw roll of 10 cms. diameter.

| Yarn used (drawn denier given) | Angle of threadline to flange ( $\theta$ ) | Snubbing pin  | Pin temperature before yarn was drawn thereon, °C. | Draw roll surface speed in ft./minute | Wind up speed in ft./minute | Twist liveliness in turns per inch |
|--------------------------------|--------------------------------------------|---------------|----------------------------------------------------|---------------------------------------|-----------------------------|------------------------------------|
| 15 denier 3 filaments          | 13°                                        | 3/16" ceramic | 21                                                 | 1,000                                 | 940                         | 0.9                                |
|                                | 7°                                         | 3/16" ceramic | 21                                                 | 2,125                                 | 2,100                       | 0.8                                |
|                                | 10°                                        | 3/16" ceramic | 21                                                 | 1,000                                 | 970                         | 1.6                                |
|                                | 21°                                        | do            | 21                                                 | 3,000                                 | 2,950                       | 2.7                                |
| 30 denier 10 filaments         | 13°                                        | do            | 21                                                 | 3,000                                 | 2,950                       | 1.1                                |
|                                | 9°                                         | do            | 21                                                 | 3,000                                 | 2,950                       | 0.75                               |
|                                | 5°                                         | 3/4" metal    | 200                                                | 3,000                                 | 2,950                       | 2.3                                |
|                                | 3°                                         | do            | 200                                                | 3,000                                 | 2,950                       | 0.9                                |
| 40 denier 13 filaments         | 8°                                         | 3/16" ceramic | 21                                                 | 2,600                                 | 2,525                       | 2.4                                |
|                                | 5°                                         | do            | 21                                                 | 2,600                                 | 2,550                       | 0.9                                |
|                                | 10°                                        | 3/16" ceramic | 21                                                 | 1,000                                 | 990                         | 2.1                                |
|                                | 3°                                         | 3/4" metal    | 200                                                | 1,700                                 | 1,650                       | 1.3                                |
| 45 denier 15 filaments         | 9°                                         | do            | 21                                                 | 1,700                                 | 1,670                       | 2.1                                |
|                                | 14°                                        | 3/8" ceramic  | 21                                                 | 1,750                                 | 1,725                       | 2.8                                |
|                                | 6°                                         | do            | 21                                                 | 1,750                                 | 1,725                       | 1.0                                |
|                                | 36°                                        | 3/8" ceramic  | 21                                                 | 1,600                                 | 1,550                       | 2.1                                |
| 205 denier 34 filaments        | 11°                                        | do            | 21                                                 | 1,100                                 | 1,010                       | 0.7                                |
|                                | 12°                                        | 3/4" metal    | 150                                                | 1,450                                 | 1,400                       | 1.4                                |
|                                | 18°                                        | do            | 150                                                | 1,075                                 | 1,050                       | 2.9                                |
|                                | 8°                                         | do            | 150                                                | 1,075                                 | 1,050                       | 1.0                                |

employed in all the figures where the apparatus concerned is the same or directly equivalent.

The combined drawing and torque-inducing apparatus of FIGURES 1 and 1a comprises feed roll 1 with its separator roll 3 and draw roll 5 with its separator roll 7, be-

#### Example II

The basic conditions of the example were the same as 75 those of Example I, save that the shore hardness of the

rubber flange was 79, its diameter was 9.4 cms. and cross-sectional radius of curvature 1.7, and the draw roll diameter was 6 cms.

| Yarn used (drawn denier given) | Flange surface | Angle of threadline to flange | Snubbing pin | Pin temperature (°C.) before yarn was drawn thereon | Draw roll surface speed, ft./min. | Wind up speed, ft./min. | Twist liveliness in turns per inch |
|--------------------------------|----------------|-------------------------------|--------------|-----------------------------------------------------|-----------------------------------|-------------------------|------------------------------------|
| 15 denier 3 filaments          | Polished       | 20°                           | 1/8" ceramic | 21                                                  | 1,850                             | 1,750                   | 1.8                                |
| Do                             | Matt           | 13°                           | do           | 21                                                  | 1,900                             | 1,750                   | 0.6                                |
|                                |                | 13°                           | do           | 21                                                  | 1,850                             | 1,800                   | 2.4                                |

### Example III

The basic conditions of this example were the same as those of Example I, save that the flange was of smooth chrome-plated metal, its diameter was 14.6 cms. and cross-sectional radius of curvature 2.3 cms., and the draw roll diameter was 10 cms.

URE 5. The metal snubbing-pin was heated to 96° C.; and the angle between the threadline and the flange was determined by the positioning of the adjustable ceramic

| Angle between threadline and flange, degree: | Twist liveliness in t.p.i. |
|----------------------------------------------|----------------------------|
| 8                                            | 0.5                        |
| 15                                           | 1.5                        |
| 20                                           | 2.0                        |

| Yarn used (drawn denier given) | Angle of threadline to flange | Snubbing Pin | Pin temperature (°C.) before yarn was drawn thereon | Draw roll surface speed in ft./min. | Wind up speed in ft./min. | Twist liveliness in t.p.i. |
|--------------------------------|-------------------------------|--------------|-----------------------------------------------------|-------------------------------------|---------------------------|----------------------------|
| 15 denier 3 filaments          | 10°                           | 1/4" metal   | 125                                                 | 2,000                               | 1,900                     | 2.5                        |
|                                | 14½°                          | do           | 112                                                 | 2,000                               | 1,900                     | 0.7                        |
| 30 denier 10 filaments         | 11°                           | 1/4" ceramic | 21                                                  | 3,050                               | 3,000                     | 2.1                        |
|                                | 5°                            | do           | 21                                                  | 3,050                               | 3,000                     | 1.6                        |
| 40 denier 13 filaments         | 4°                            | do           | 21                                                  | 3,050                               | 3,000                     | 0.8                        |
|                                | 17°                           | 1/4" metal   | 118                                                 | 2,600                               | 2,500                     | 2.5                        |
|                                | 11°                           | do           | 110                                                 | 2,600                               | 2,500                     | 1.6                        |
| 45 denier 15 filaments         | 7°                            | do           | 120                                                 | 2,600                               | 2,500                     | 0.8                        |
|                                | 16°                           | do           | 135                                                 | 1,700                               | 1,650                     | 2.5                        |
|                                | 15°                           | do           | 133                                                 | 1,700                               | 1,650                     | 0.5                        |
| 205 denier 34 filaments        | 20°                           | 1/4" ceramic | 21                                                  | 1,100                               | 1,050                     | 0.5                        |
|                                | 11°                           | 1/4" metal   | 230                                                 | 1,050                               | 1,000                     | 0.9                        |
|                                | 11°                           | do           | 150                                                 | 1,050                               | 1,000                     | 0.6                        |
|                                | 13°                           | do           | 110                                                 | 1,050                               | 1,000                     | 0.9                        |

### Example IV

35

In this example, multifilament yarns of polyhexamethylene adipamide, of the deniers and filament numbers indicated, were drawn and subsequently heat-relaxed in a 22-inch long hot air heater whilst torque was induced in them, by the apparatus of FIGURE 2.

| Yarn used (drawn denier given) | Draw roll speed in ft./min. | Air temperature (°C.) in heater | False twist head speed in r.p.m. $\times 10^4$ | Wind up speed in ft./min. | Twist liveliness in t.p.i. |
|--------------------------------|-----------------------------|---------------------------------|------------------------------------------------|---------------------------|----------------------------|
| 15 denier 3 filaments          | 2,000                       | 230                             | 13                                             | 1,850                     | 2.1                        |
| 45 denier 15 filaments         | 2,000                       | 215                             | 16                                             | 1,750                     | 1.8                        |

### Example V

45 denier 15 filament yarn of polyhexamethylene adipamide was drawn and subsequently heat-relaxed in an 8% relaxation step whilst torque was induced in it using the apparatus of FIGURE 3. The two heating surfaces of the "pyramid" heater were each 6 inches long.

| Draw roll speed in ft./min. | Contact heater surface temperature in °C. | False twist head speed in r.p.m. $\times 10^4$ | Wind up speed in ft./min. | Twist liveliness in t.p.i. |
|-----------------------------|-------------------------------------------|------------------------------------------------|---------------------------|----------------------------|
| 1,070                       | 150                                       | 18                                             | 985                       | 0.5                        |
| 1,070                       | 230                                       | 18                                             | 985                       | 2.5                        |

### Example VI

45 denier 15 filament yarn of polyhexamethylene adipamide was false twisted whilst being drawn, using the apparatus of FIGURE 4. The contact heater was 24 inches long; and the yarn was drawn at 800 feet/minute.

| Heater temperature in °C. | False twist head speed in r.p.m. | Twist liveliness in resultant yarn in t.p.i. |
|---------------------------|----------------------------------|----------------------------------------------|
| 130                       | 300,000                          | 0.5                                          |
| 180                       | 300,000                          | 2.3                                          |
| 230                       | 130,000                          | 0.5                                          |

### Example VII

150 denier 30 filament yarn of "Terylene" (registered trademark) polyester fibre was drawn at 2,130 feet/minute and torque was induced in it by the apparatus of FIG-

4% to 6%, was satisfactory for use in the welts of stockings when twist of 0.25 turn per inch was inserted by the twister wind-up and torque from 0.3 to 0.7 turn per inch in the same direction as the twist was induced by the false twister, whereby the speed of production was significantly raised in comparison with the standard process in which it was necessary to impart 0.6–0.7 turn per inch twist.

55 What I claim is:

1. A compact, synthetic multifilament yarn having no crimp and no substantial unidirectional twist, characterized in that the yarn has a unidirectional torque from 0.25 to 2.5 turns per inch and that the filaments are substantially parallel to one another and to the length direction of the yarn.

2. A compact, synthetic multifilament yarn, characterized in that the yarn has a unidirectional twist of not greater than 0.25 turn per inch and a torque of from 0.25 to 2.5 turns per inch in the same direction as the said twist.

3. A compact, synthetic multifilament yarn according to claim 1 and having a residual shrinkage not greater than half its normal value.

4. A compact, synthetic multifilament yarn according to claim 2, in which the filaments are of poly-hexamethylene adipamide having a residual boiling water shrinkage of between 4% and 6%.

| References Cited                  |         |                  |             |
|-----------------------------------|---------|------------------|-------------|
| UNITED STATES PATENTS             |         |                  |             |
| 2,771,660                         | 11/1956 | Ephland          | 57—157 XR   |
| 2,777,310                         | 1/1957  | Comer.           |             |
| 2,796,655                         | 6/1957  | Stuewer          | 57—140 XR 5 |
| 3,035,396                         | 5/1962  | Biggers          | 57—34       |
| 3,041,814                         | 7/1962  | Held             | 57—34       |
| 3,091,912                         | 6/1963  | Stoddard et al.  | 57—34 XR    |
| 3,196,602                         | 7/1965  | Jenkins et al.   | 57—34 XR    |
| 2,952,964                         | 9/1960  | Gonsalves et al. | 57—34 10    |
| 3,001,355                         | 9/1961  | Evans            | 57—34       |
| 3,069,837                         | 12/1962 | Olson            | 57—34 XR    |
| 3,094,834                         | 6/1963  | Deeley et al.    | 57—157 XR   |
| 3,137,119                         | 6/1964  | Crouzet          | 57—157      |
| 3,292,354                         | 12/1966 | Chalfant et al.  | 57—34       |
| 3,330,104                         | 7/1967  | Dunwoody         | 57—106 XR   |
| FRANK J. COHEN, Primary Examiner. |         |                  |             |
| D. WATKINS, Assistant Examiner.   |         |                  |             |